

## UNITED STATES PATENT OFFICE

2,187,388

## WORKING FLUID FOR REFRIGERATING APPARATUS

Harry M. Williams, Dayton, Ohio, assignor to  
General Motors Corporation, Dayton, Ohio, a  
corporation of Delaware

No Drawing. Application September 6, 1935,  
Serial No. 39,453

9 Claims. (Cl. 252—5)

This application is a continuation-in-part of my two co-pending applications, Serial No. 465,029, filed June 30, 1930, and Serial No. 524,-409, filed March 21, 1931.

This invention relates to refrigeration and more particularly to working fluids for refrigerating apparatus having working parts requiring lubrication within a refrigerant circuit.

Heretofore it has been customary to use as working fluids in mechanical refrigerating systems a mixture of a refrigerant such as sulphur dioxide or ammonia with a mineral oil which is immiscible for the most part with these refrigerants. Refrigerating apparatus has been designed for use with such a working fluid and difficulties are often encountered with such refrigerating systems when such working fluids are not used. When it is desired to use a non-toxic, non-inflammable refrigerant such as one of the fluorine derivatives of the aliphatic hydrocarbons such as the familiar difluorodichloro-methane and the tetrafluorodichloro-ethane, difficulty has been encountered because of the fact that mineral oil is completely immiscible in all proportions with this class of refrigerants.

It is an object of my invention to provide non-toxic, non-inflammable working fluids for refrigerating systems having lubricants which are wholly or partially immiscible with the refrigerants.

More specifically it is an object of my invention to provide a working fluid containing one of the derivatives of aliphatic hydrocarbons, for example, difluorodichloro-methane or tetrafluorodichloro-ethane with a lubricant where is wholly or partially immiscible therewith.

As one example of my invention, I employ difluorodichloro-methane and castor oil as a working fluid or charge for a refrigerating system. These two fluids have a relatively small mutual miscibility or solubility and when sufficient castor oil is provided in proportion to the difluorodichloro-methane, this working fluid forms two layers or phases of liquid.

I have found that difluorodichloro-methane and castor oil have a limited affinity for each other so that only a small quantity of castor oil will disappear into the body of the refrigerant, the remainder being free in this case as a layer or phase on top of the refrigerant. There is usually a relatively small mutual immiscibility or solubility between the lubricant and the refrigerant, and there may be a slight amount of refrigerant dissolved in the upper lubricant layer on top of the body of the refrigerant. In this upper layer

or phase the lubricant greatly predominates since such upper layer or phase is essentially an oily body, it is termed herein a free lubricant.

In the use of this working fluid, the content of the castor oil in proportion to the difluorodichloro-methane may be readily controlled so that for any particular type of machine the free lubricant is of such a quality as desired for the best operation of the refrigerating machine. This gives several benefits in operation such as high efficiency and in service the relative quantities of lubricant and refrigerant may be more readily determined as in cases where additional changing is necessary.

As another specific example of a working fluid embodying my invention I provide a fluid comprising tetrafluorodichloro-ethane and castor oil. These substances likewise have only a limited affinity for each other so that only a small quantity of castor oil will disappear into the refrigerant, and the remainder forming a layer on top of the refrigerant containing a slight amount of refrigerant dissolved therein. This upper layer is essentially an oily body, and is termed herein a free lubricant.

Preferably the castor oil used in the before mentioned working fluid is one which has been dewaxed by cooling the oil to extremely low temperatures by refrigeration until the wax solidifies and then separating the liquid castor oil from the wax. If the castor oil used in these working fluids containing either difluorodichloro-methane and castor oil or tetrafluorodichloro-ethane and castor oil has not been dewaxed, I add a solvent for the wax such as methyl or ethyl alcohol in sufficient quantities to prevent the wax from solidifying or becoming excessively viscous at the lowest temperatures encountered in the refrigerating system in which the working fluid is to be used.

As another specific example of my invention I provide a working fluid comprising difluorodichloro-methane and glycerine. This working fluid likewise forms two layers, the one layer or phase being essentially an oily body, termed herein a free lubricant, while the other layer forms a refrigerant.

As another specific example of my invention I provide a working fluid comprising tetrafluorodichloro-ethane and glycerine which likewise forms two phases, one of these phases or layers is an oily body, termed herein a free lubricant.

Preferably, I use chemically pure glycerine. However, if the glycerine contains wax, I add a solvent for the wax such as ethyl or methyl al-

cohol in sufficient quantities to prevent the wax from congealing in the refrigerating system.

As another specific example of my invention I provide a working fluid comprising difluorodichloro-methane and diethylene glycol. This working fluid likewise forms two phases, one of which is a lubricant phase.

Another example of my invention is a working fluid comprising tetrafluorodichloro-ethane and diethylene glycol, which likewise forms two phases or layers, one of which is a lubricant phase.

While I have mentioned specifically difluorodichloro-methane and tetrafluorodichloro-ethane as refrigerants which are not miscible with the lubricants mentioned namely in castor oil, glycerine and diethylene glycol, these refrigerants are merely specific examples of the large class of refrigerants which are fluoro derivatives of aliphatic hydrocarbons to which the present invention is applicable. Of this class of refrigerants, I prefer to employ the halofluoro derivatives of the aliphatic hydrocarbons which contain both fluorine and another halide.

The working fluids disclosed are particularly adaptable for use in refrigerant apparatus wherein the refrigerant is mechanically compressed, condensed and evaporated. In the so-called flooded type refrigerating system, a small amount of lubricant is carried in solution in the condensed refrigerant to the flooded evaporator and the evaporation of the refrigerant concentrates the lubricant content of the fluid in the evaporator to such an extent that a layer or phase of free lubricant separates from the refrigerant. This free lubricant in such a system is returned to the compressor along with the refrigerant by the use of some kind of device in the evaporator for withdrawing the free lubricant from this phase.

The direct expansion type of refrigerant apparatus and method, the condensed refrigerant carrying a slight amount of lubricant is expanded into a confined tube of a substantially uniform diameter where the velocity of the evaporated refrigerant sweeps the separated lubricant back into the compressor.

In these two types of refrigerant apparatus, and in methods above mentioned, as well as other types of apparatus, and methods, any lubricant discharged by the compressor may be separated from the compressed but uncondensed refrigerant or from the compressed and condensed refrigerant, and returned to the compressor before a condensed refrigerant is discharged into the evaporator.

While the form of embodiment of the present invention constitutes a preferred form, it is to be understood that other forms might be adopted, all coming within the scope of the claims which follow.

What is claimed is as follows:

1. A refrigerating fluid comprising a halofluoro derivative of an aliphatic hydrocarbon and castor oil.
2. A refrigerating fluid comprising dichlorodifluoro methane and castor oil.
3. A working fluid for a compression refrigerating system comprising a fluoro derivative of an aliphatic hydrocarbon and castor oil.
4. A refrigerating medium comprising difluorodichloromethane and castor oil free from superfluous wax.
5. A refrigerating medium comprising difluorodichloromethane, castor oil containing a wax, and a solvent for the wax.
6. A refrigerating medium comprising difluorodichloromethane, castor oil, and alcohol.
7. A working fluid for a compression refrigerating system comprising a fluoro derivative of an aliphatic hydrocarbon and glycerine.
8. A working fluid for a compression refrigerating system comprising a fluoro derivative of an aliphatic hydrocarbon and diethylene glycol.
9. A refrigerating medium comprising a halofluoro derivative of an aliphatic hydrocarbon and a liquid substantially immiscible therewith and having lubricating properties, said liquid being selected from a group of lubricants consisting of castor oil and a polyhydric alcohol having a low pour point and a high vaporization temperature.

HARRY M. WILLIAMS.